

Oct. 8, 1940.

H. SCOTT

2,217,423

GLASS-TO-METAL SEAL

Original Filed April 30, 1936

Fig. 1.



Fig. 2.



WITNESSES:

Leon J. Faga  
G. J. Bryant

INVENTOR

Howard Scott.

BY

Frank Savage

ATTORNEY

## UNITED STATES PATENT OFFICE

2,217,423

## GLASS-TO-METAL SEAL

Howard Scott, Forest Hills, Pa., assignor to Westinghouse Electric & Manufacturing Company, East Pittsburgh, Pa., a corporation of Pennsylvania

Application April 30, 1936, Serial No. 77,221  
Renewed July 17, 1940

2 Claims. (Cl. 48—92)

This application is a continuation-in-part of my application Serial No. 376,291, filed July 5, 1929, now Patent 2,062,335 granted Dec. 1, 1936, and relating to seals between metal and glass.

5 My invention relates to vacuum-tight seals and it has particular relation to seals between electrical insulating materials of the class typified by glass and metallic compositions of the class typified by ferrous base alloys.

10 For many applications of vacuum-tight joints of the character named, the use of a hard or boro-silica glass is of advantage. The high "strain point" or temperature at which such a glass will first begin to soften permits the assembled apparatus to be "treated out" under high temperature vacuum conditions without danger of collapse. In effect, the strain point represents the lower limit of the customary annealing range of the glass.

15 20 Iron-base alloys are of especial advantage in glass-sealing applications because of their low cost, easy fabrication, immunity from attack by mercury, and ability to "wet" glass. Such alloys may be compounded from iron, nickel and cobalt to have mean expansivities very closely matching those of the described hard glass from a static or room temperature up to the "inflection" temperature of the alloy.

25 30 As above used, the term "static" designates the lower limit of the temperature range to which the seal is in service to be subjected and the term "inflection" designates the temperature above which the expansivity of the alloy increases rapidly. The point of this abrupt rise in coefficient 35 of expansion of the metal may, in the case of the ferrous base composition above mentioned, be made to approach the strain point of commercially available grades of hard glass. It is only above the strain point that stresses from the differential expansion between the metal and glass 40 can be relieved substantially by plastic flow.

45 50 These iron-base alloys, however, are further characterized by having expansion-temperature curves which decrease in slope as the temperature rises above room or static value and then start again to rise more rapidly as the inflection temperature is approached. The expansion curve of hard glass, on the other hand, is substantially linear in form within the range of temperatures below the strain point.

55 Typically, therefore, the curve of an iron-base alloy of comparable mean expansivity will cross and recross that of hard glass. Such a condition is contrary to the past accepted theory of glass-to-metal seals—that both the glass and the metal

should have the same coefficient of expansion for each degree up to the annealing range of the glass. In the light of this theory, others have predicted many practical difficulties in sealing ferrous-base alloys into hard glass.

5 I have discovered that these difficulties are by no means insurmountable and that exact identity of expansion per degree up to the annealing range of the glass is not necessary between the glass and the metal if the overall expansions of the materials between static or room temperature and the strain point of the glass are substantially the same. In accordance with my discovery I am able to make satisfactory seals between the two materials named.

10 15 My invention will best be understood through the following description of two specific embodiments represented by Figs. 1 and 2 of the accompanying drawing.

20 In Fig. 1, I have represented at 10 the expansion-temperature curve of one composition of hard glass known as "Meth" and at 12 the corresponding curve of a ferrous-base alloy which I have found to produce a satisfactory seal with this glass. This alloy is composed of 31.9% of 25 nickel, 9.8% of cobalt, 0.79% of manganese, 0.01% of carbon and the remainder of 57.4% of iron.

25 30 It will be noted that whereas curve 10 is substantially a straight line, curve 12 is sufficiently irregular in shape to cross and recross at points 14 and 16, respectively. Between the strain point 18 of the glass and the static or room temperature, however, the overall expansivities of the two materials are substantially the same. The differences at intermediate temperatures are, I have discovered, insufficient to produce strains of an objectionable or disruptive nature.

35 40 In Fig. 2, I have represented a different combination of sealable materials. Curve 20 applies to "G-80" glass composed of 72.4%  $\text{SiO}_2$ ; 10.2%  $\text{B}_2\text{O}_3$ ; 9.8%  $\text{Na}_2\text{O}$ ; 5.10%  $\text{Al}_2\text{O}_3$ ; 1.75%  $\text{PbO}$ ; and 0.40%  $\text{K}_2\text{O}$ .

45 50 Curve 22 applies to a ferrous-base alloy suitable for sealing into this glass, which alloy is made up 31.8% of nickel, 16.0% of cobalt, 0.65% of manganese, 0.01% carbon and the remainder of iron.

55 In the combination represented in Fig. 2, curve 22 also crosses curve 20 of the glass at two points, 50 54 and 56. The overall expansion, however, between the strain point 58 of the glass and the static or room temperature is substantially the same for the two materials and no damaging stresses are set up at intermediate temperatures. 55

It will be obvious that other equivalent combinations of glass and ferrous-base alloys complying with this condition may be successfully joined. My invention, therefore, is not to be restricted except insofar as is necessitated by the prior art and by the scope of the appended claims.

I claim as my invention:

- 5 1. A glass-to-metal thermal joint in which the glass has an overall expansion between the static temperature of the joint and the strain point of the glass substantially the same as that of the

metal between these temperatures and a coefficient of expansion substantially different from the metal at an intermediate temperature.

2. A vacuum-tight seal between a ferrous-base alloy and a glass having an overall expansion between the static temperature of the seal and the strain point of the glass substantially the same as that of the alloy for the same range of temperatures and a thermal coefficient of expansion different from that of the alloy at an intermediate temperature.

10 HOWARD SCOTT.